

## UNITED STATES PATENT OFFICE

2,527,268

## PRODUCTION OF PHOTOGRAPHIC EMULSIONS

John Alfred Henry Hart, Ottawa, Ontario, Canada, and Kenneth George Alfred Pankhurst, Brentwood, and Robert Charles Morris Smith, Ilford, England, assignors to Ilford Limited, Ilford, England, a British company

No Drawing. Application March 30, 1949, Serial No. 84,486. In Great Britain October 30, 1944

8 Claims. (Cl. 95—7)

2

This invention relates to the production of silver halide photographic emulsions.

It has been discovered that when there is added to an emulsion of silver halide in gelatin, at a low pH value, a sulphonic acid containing a highly hydrophobic radicle in the anion, a complex is formed between the gelatin and sulphonic acid and this separates out carrying the silver halide with it. It has further been discovered that complexes thus formed are readily dispersible in organic solvents, e. g. methyl alcohol. The term "sulphonic acid" is to be understood to include sulphonates. According to this invention, therefore, photographic emulsions in which the solvent medium is predominantly organic are formed by dispersing in an organic solvent medium a complex formed by precipitating gelatin from its aqueous dispersion containing silver halide in suspension, by means of a sulphonic acid containing a highly hydrophobic radicle in the anion, the said aqueous dispersion being at a pH value below the isoelectric point of the gelatin. The precipitated complex may contain a small proportion of water and this be included in the organic solvent dispersion.

According to a further feature of the invention, there is included in a photographic emulsion so formed a proportion of another colloid which is soluble in the solvent medium already present in the emulsion, or which is soluble in a solvent medium which is miscible with the solvent medium already present in the emulsion, to form a stable combination.

The gelatin/sulphonate complexes containing silver halide may be prepared by the addition of the sulphonic acid or sulphonate solution to the gelatin silver halide emulsion and allowing the gelatin complex to sediment out. The complexes may be redispersed in the organic solvent medium without washing, but it is preferred to wash the complex to remove unwanted ions. Instead of the sulphonic acid itself it is preferred to use the corresponding soluble salts owing to the relative insolubility of the free acids.

The quantity of sulphonic acid or sulphonate employed relative to the gelatin may vary, but there is no advantage to be gained by using a quantity greater than the stoichiometric equivalent, i. e. about 10 mgm. moles per gram of dry gelatin.

For emulsion-making it is generally desirable that the precipitated gelatin/sulphonate complex should be soluble in water-miscible solvents since the precipitated complex invariably contains water, and it is difficult to remove this water without adversely affecting the quality of the emulsion. To this end it is generally desirable to treat the emulsion at a pH below the isoelectric point of the gelatin and in the presence of as little electrolyte as possible.

Any sulphonic acid of which the alkali or ammonium salt is soluble in water and of which the anion is highly hydrophobic may be employed. These may be simple acids, for example naphthalene-2-sulphonic acid, naphthalene 1,5-disulphonic acid, naphthalene 1:3:5-tri-sulphonic acid, 2-naphthol-1-sulphonic acid, 2-naphthol-6-sulphonic acid, 1-naphthol-4-sulphonic acid, 1-naphthol-3:6-disulphonic acid or anthraquinone-2-sulphonic acid, or may be more complex, for example dyestuffs such as Kiton Fast Yellow 3G (Colour Index No. 645) which contains a sulphonyl-pyrazolone radicle; Naphthalene Orange GS (Imperial Chemical Industries Ltd.) and Tartrazine.

In general it is preferred to form the complex from an aqueous gelatino-silver halide emulsion which has already been washed and digested.

Generally speaking, the most suitable organic solvents for dispersing the complexes are those containing hydroxy groups, e. g. methyl and ethyl alcohols, ethylene glycol mono methyl ether, ethyl lactate and diacetone alcohol. Organic solvents not containing hydroxy groups are generally only useful together with some water or some hydroxy solvent, e. g. acetone, methyl ethyl ketone, dioxane, methylene chloride, chloroform and mesityl oxide are preferably used in admixture with water or methyl alcohol. Small quantities of esters, e. g. methyl acetate, butyl acetate, ethers, e. g. diethyl ether, and hydrocarbons, e. g. benzene and toluene, may also be included in the solvent medium. The choice of solvent will depend on the particular nature of the complex. Solubility in toluene and chloroform appears to increase the greater the quantity of the sulphonate relative to gelatin. The complexes may be swollen in the organic solvent medium and dispersion is usually facilitated by gentle warming.

The following table shows examples of the preferred conditions for precipitating a gelatin/sulphonate complex using various sodium sulphonates.

| Sulphonic Acid (sodium salt)            | Quantity added per gram of gelatin | Solubility characteristics of the precipitated complex |         |
|-----------------------------------------|------------------------------------|--------------------------------------------------------|---------|
|                                         |                                    | Grams                                                  | Toluene |
| (a) naphthalene-2-sulphonic acid        | 2.3                                | s                                                      | vs      |
| (b) naphthalene-1,5-disulphonic acid    | 1.61                               | s                                                      | vs      |
| (c) naphthalene-1,3,5-trisulphonic acid | 1.44                               |                                                        | ss      |
| (d) 2-naphthol-6-sulphonic acid         | 1.24                               |                                                        | s       |
| (e) 1-naphthol-3:6-disulphonic acid     | 1.1                                |                                                        | s       |
| (f) Tartrazine                          | 1.0-2.0                            | i                                                      | vs      |

60 s=soluble; vs=very soluble; ss=slightly soluble; i=insoluble.

Referring to this table, complex (a) in solution in aqueous alcohol is not precipitated by the addition of excess alcohol and this complex is also very soluble in carbon tetrachloride, acetone and ethyl acetate. Complex (b) in solution in aqueous alcohol is precipitated by the addition of excess alcohol and this complex is also soluble in ethyl acetate and very soluble in acetone; the same remarks apply to complex (c). Complex (e) in solution in aqueous alcohol is precipitated by excess alcohol, and complex (f) in solution in aqueous alcohol is precipitated by the addition of excess water.

In the preparation of the complexes referred to in this table the gelatin concentration was 0.5% and the temperature was 35° C. in each case.

As already indicated, an important feature of this invention is the formation of photographic emulsions which comprise a gelatin/sulphonate complex, containing silver halide, dispersed in an organic solvent medium, together with a proportion of another colloid soluble in such organic solvent medium or in an organic solvent medium miscible therewith. Such other colloids may be, for example, cellulose esters, e. g. cellulose nitrate, cellulose acetate, far-hydrolysed cellulose esters (e. g. cellulose acetate having an acetyl content of 20 to 30%), polyvinyl acetates, polyvinyl acetals, methyl methacrylate polymers and the partial hydrolysis products thereof, alkyd resins, and mixed interpolymers such as the interpolymers of maleic acid or anhydride with styrene or methyl methacrylate.

The following examples illustrate the invention, but are not to be regarded as limiting it in any way:

*Example I*

1000 cc. of an aqueous gelatino silver bromide emulsion containing 11% gelatin and 17% silver bromide was brought to pH 2.0-2.4 by addition of 10 cc. concentrated hydrochloric acid. To this was added 400 cc. of an 8% solution in water of sodium 2-naphthalene monosulphonate. The gelatin/sulphonate complex (containing suspended silver bromide) separated as a stiff oily complex. The supernatant liquid was decanted and the complex dissolved in warm methyl alcohol to form a 7% solution. This was a satisfactory photographic emulsion and could be coated in the usual way. Its sensitometric characteristics were substantially the same as those of the original aqueous gelatin emulsion from which it was obtained.

*Example II*

To a photographic emulsion in methyl alcohol obtained in Example I was added, in turn:

|                                                                  |    |     |
|------------------------------------------------------------------|----|-----|
| Ethylene glycol mono-methyl ether                                | cc | 400 |
| Low viscosity cellulose nitrate (10% solution in methyl alcohol) | cc | 300 |
| Acetone                                                          | cc | 400 |

The final emulsion so obtained was stable and suitable for coating by the usual techniques. It was especially suitable, however, for coating by the spray-coating technique. It had a suitable viscosity for this purpose and could be sprayed on to cellulose nitrate lacquered metal without the need for any special substratum or anchoring layer since it adhered strongly to the lacquer coating both in the dry condition and during all stages of processing. The emulsion developed normally, and it was found that the coating was not melted by hot water.

Although in the above Example I the precipitated complex was re-dispersed in methyl alcohol to form an emulsion for coating, other water-miscible solvents may be used, for example ethyl alcohol and ethylene glycol monomethyl ether.

The silver halide emulsions of this invention may contain any of the usual additions to silver halide emulsions, e. g. optical sensitising dyes, sulphur sensitisers as for instance allyl isothiocyanate, gold salts as described in U. S. P. 2,399,-083, stabilisers, anti-fogging agents, toning agents and other agents for modifying the speed, contrast, graininess, fog level and image colour of the products.

The invention provides photographic emulsions having a gelatin basis dispersed in organic solvent and the emulsions are therefore of value in a number of special applications. As already indicated they are of particular value for spray coating. Normal gelatin silver halide emulsions present considerable difficulties in spray coating since it is usually necessary to maintain the emulsion warm in the spray-gun to prevent it setting therein. Moreover, the ordinary emulsions will not adhere firmly if sprayed on to lacquered metal sheet. Emulsions may be prepared according to this invention, however, which have little tendency to set in the spray-gun. Moreover, the organic solvent usually has a slight solvent action on lacquered surfaces and thus facilitates adhesion between such surfaces and the emulsion sprayed thereon.

The spray-coating of lacquered metal sheets with photographic emulsion is of particular value in the production of photo-templates. In the commercial application of this process, however, the users generally prefer that the emulsion should be supplied in dry granular condition so that it may be re-dispersed when required to form an emulsion suitable for spraying. The present emulsions are especially suitable in this connection. Emulsions prepared in organic solvent media according to this invention can easily be derived by the well-known expedients of film drying, spray drying, and air drying of the emulsion in the form of a shredded set jelly, since the organic solvent readily evaporates. A further method is to precipitate the emulsion by adding it to water and, after breaking up the precipitate, to air-dry the product.

The emulsions of this invention, either as originally prepared or as re-constituted after drying, can be used in any process where spray-coating is required. The production of photo-templates has already been mentioned, and another useful application is in the preparation of dials, nameplates and the like on metal or other surfaces. A further application is in the preparation of silk-screen printing surfaces. In this application the emulsion is sprayed on to stretched silk, dried, exposed, developed in a tanning developer and washed in hot water to produce a wash-out relief image. It is a peculiar characteristic of the emulsions of this invention that, though quite insoluble in water when coated, they tend to become soluble when allowed to stand in contact with alkali, as in normal development, though the emulsions are still not soluble in water except at high temperatures. Fixing in an acid fixing bath, however, restores the insolubility of the complex even in hot water. Thus a suitable technique for using the emulsions in the production of silk-screen relief images is to develop the exposed image in alkaline pyrocatechol, plunge the silk into hot water and then to fix the wash-out

relief image. An alternative technique is to prepare the wash-out relief image on a support from which it may be stripped and to transfer the image to a silk support.

The emulsions of this invention are also of value in colour photography. Thus they may contain dyes or dye-intermediates, e. g. colour-formers which react with the oxidation products of aromatic primary amino developing agents to form quinone-imine or azo-methine dyes, the colour-former being uniformly dispersed in the emulsion. The colour-former, especially where particulate or of very high molecular weight, may be included in the original emulsion and precipitated with the complex, or it may be added to the final emulsion. Many of the high-molecular weight colour-formers, which are preferred from the standpoint of being non-diffusing in the emulsion, are difficult to disperse in ordinary aqueous gelatin silver halide emulsions, but more easily dispersed in the organic solvent emulsions of this invention.

The emulsions of this invention are permeable to ordinary alkaline developers, but the degree of permeability depends on the precise constitution of the emulsion. By a suitable selection of an additional colloid, e. g. cellulose nitrate or a hydrophobic acid colloid, emulsions of varying degree of developer-permeability may be made, and accordingly it is possible to build up a multilayer photographic material for colour photography in which the several layers have different degrees of permeability to ordinary developers and, by adjusting the constitution of the developers, e. g. by adding organic solvents, to develop each of the layers separately. In such a process, by using aromatic primary amino developing agents containing different colour-formers, images in different colours may be formed in the various layers, and by a suitable selection of colour-formers a final true-colour image may be obtained.

Another use to which the emulsions of this invention may be put is in the production of printing paper to be used for printing from wet negatives. As already stated the emulsions of this invention have a good resistance to water, though they are readily developed by ordinary alkaline developing solutions. Paper coated with emulsion according to this invention may be used for printing from wet negatives, though it is usually desirable to employ an emulsion containing a proportion of other colloids, e. g. cellulose nitrate and a methyl methacrylate-methacrylic acid co-polymer. Such emulsions not only have a good resistance to water but also a good resistance to hypo, which may be carried by the wet negative. Advantageously, in the production of wet-printing paper using the emulsions of this invention the emulsion should be supercoated with a layer of a plain gelatin/anion soap complex in organic solvent, as described in our co-pending application Serial No. 623,446, or a plain gelatin/sulphonate complex in organic solvent as described in co-pending application Serial No. 84,485, filed March 30, 1949, which is a continuation-in-part of application No. 623,446.

What we claim is:

1. A photographic emulsion containing a complex of gelatin and a sulphonic acid containing a highly hydrophobic radicle in the anion, said complex being soluble in a solution composed of methyl alcohol and containing dispersed silver halide, dispersed in a predominantly organic solvent medium.

2. A photographic emulsion containing a com-

plex of gelatin and a sulphonic acid containing a highly hydrophobic radicle in the anion, said complex being soluble in a solution composed of methyl alcohol and containing dispersed silver halide, dispersed in a predominantly organic solvent medium, said emulsion further containing a proportion of another colloid which is soluble in the said solvent medium.

3. A photographic emulsion containing a complex of gelatin and a sulphonic acid containing a highly hydrophobic radicle in the anion, said complex being soluble in a solution composed of methyl alcohol and containing dispersed silver halide, dispersed in a predominantly organic solvent medium containing methyl alcohol.

4. A photographic emulsion containing a complex of gelatin and a sulphonic acid containing a highly hydrophobic radicle in the anion, said complex being soluble in a solution composed of methyl alcohol and containing dispersed silver halide, dispersed in a predominantly organic solvent medium containing methyl alcohol and acetone, said emulsion further containing a proportion of another colloid which is soluble in the said solvent medium.

5. A photographic emulsion containing a complex of gelatin and a naphthalene mono sulphonate acid, said complex being soluble in a solution composed of methyl alcohol and containing dispersed silver halide, dispersed in a predominantly organic solvent medium.

6. A photographic emulsion containing a complex of gelatin and a naphthalene mono sulphonate acid, said complex being soluble in a solution composed of methyl alcohol and containing dispersed silver halide, dispersed in a predominantly organic solvent medium, said emulsion further containing a proportion of another colloid which is soluble in the said solvent medium.

7. A photographic emulsion containing a complex of gelatin and a naphthalene mono sulphonate acid, said complex being soluble in a solution composed of methyl alcohol and containing dispersed silver halide, dispersed in a predominantly organic solvent medium containing methyl alcohol.

8. A photographic emulsion containing a complex of gelatin and a naphthalene mono sulphonate acid, said complex being soluble in a solution composed of methyl alcohol and containing dispersed silver halide, dispersed in a predominantly organic solvent medium containing methyl alcohol and acetone, said emulsion further containing a proportion of another colloid which is soluble in the said solvent medium.

JOHN ALFRED HENRY HART.

KENNETH GEORGE ALFRED PANKHURST.  
ROBERT CHARLES MORRIS SMITH.

REFERENCES CITED

The following references are of record in the file of this patent:

UNITED STATES PATENTS

| Number    | Name          | Date          |
|-----------|---------------|---------------|
| 1,290,794 | Sheppard      | Jan. 7, 1919  |
| 2,142,311 | Heidenhain    | Jan. 3, 1939  |
| 2,304,940 | Mannes et al. | Dec. 15, 1942 |
| 2,489,341 | Waller et al. | Nov. 29, 1949 |

FOREIGN PATENTS

| Number  | Country       | Date         |
|---------|---------------|--------------|
| 556,360 | Great Britain | Oct. 1, 1943 |

